

# UNITED STATES PATENT OFFICE.

DAVID MACINTOSH, OF NEWARK, NEW JERSEY.

## ART OF ANNEALING METAL CASTINGS.

1,356,644.

Specification of Letters Patent. Patented Oct. 26, 1920.

No Drawing.

Application filed July 11, 1919. Serial No. 310,128.

To all whom it may concern:

Be it known that I, DAVID MACINTOSH, of Newark, in the county of Essex and State of New Jersey, have invented a certain new 5 and useful Improvement in the Art of Annealing Metal Castings, of which improvement the following is a specification.

This invention relates to the art of annealing castings, and more particularly the 10 process of making malleable iron castings, the object being to provide an improved packing material in which the castings are embedded during the heating operation for furnishing the necessary oxygen for 15 carbonization, and at the same time prevent the castings from fusing or sticking to the packing material or to one another when the same are taken out after cooling.

Heretofore it has been customary to use 20 an iron oxid, such as metal filings or borings, as a packing material for cast iron articles in annealing the same to produce malleable castings, in which operation, under the high temperature, some of the oxygen 25 of the ferric oxid combines with carbon from the casting, thus forming carbonic oxid, which passes off as gas, and effects the desired decarbonization of the outer portion of the casting. Under the high temperature, however, the packing material fuses 30 more or less with the castings, so that after cooling, many of the castings are found stuck together in a mass, which can be separated only with difficulty. It then requires 35 considerable time and effort to break the masses apart, separate and clean up the castings, all of which causes delay and increases the cost of manufacture. These objections are overcome by means of my im- 40 proved packing material, which does not fuse or stick to the malleable castings, but falls freely away from the same when taken out after cooling, leaving the castings perfectly clean.

According to the practice of my invention, the iron castings to be annealed are packed in the heating boxes, filled with calcium carbonate, preferably in the form of 45 ground shells, such as oyster shells, the same 50 being packed in layers between the layers of castings which are embedded therein, so that there is a large amount of the calcium car-

bonate relative to the iron. The loaded boxes are then placed in the oven and heated to a high temperature of about 1600 to 55 1700 degrees Fahrenheit, and held at that temperature for a certain period of time, usually about three or four hours, after which they are gradually cooled and then taken out. 60

When the boxes are emptied, the castings readily separate from the packing material, which falls away, leaving the clean castings with no tendency to stick together. The malleable castings are also found to be thoroughly annealed and may be pounded and bent without breaking, thus showing the efficiency of the process. 65

The packing material of oyster shells may also be used over again for several times, 70 and is then reduced to quick lime, CaO, which is itself a valuable by-product, and may be sold for various purposes.

My improvement has the advantage of greatly reducing the time and expense involved in making malleable iron castings, 75 as the packing material employed, *i. e.*, oyster shells, is very cheap, being now thrown away in large quantities at wharves and markets, where they can be had for 80 nothing by simply carting them away.

Having now described my invention, what I claim as new and desire to secure by Letters Patent is:

1. The process of annealing castings, 85 which consists in embedding said castings in a packing material consisting wholly of calcium carbonate in granular form, and in a large quantity relative to the amount of iron, heating the same to a high temperature for a period of time, and then gradually cooling the same. 90

2. The process of annealing castings, 95 which consists in embedding said castings in a packing material consisting wholly of ground oyster shells, there being a large amount of said packing material relative to the amount of iron, heating the same to a high temperature for a period of time, and then gradually cooling the same. 100

In testimony whereof I have hereunto set my hand.

DAVID MACINTOSH.